

Patented Sept. 29, 1931

1,824,837

# UNITED STATES PATENT OFFICE

GEORGE A. RICHTER, OF BERLIN, NEW HAMPSHIRE, ASSIGNOR TO BROWN COMPANY,  
OF BERLIN, NEW HAMPSHIRE, A CORPORATION OF MAINE

## PAPERMAKING COMPOSITION

No Drawing.

Application filed November 15, 1929. Serial No. 407,589.

This invention relates to papermaking compositions, being more particularly concerned with compositions which may be used in making high grade papers having a combination of desirable characteristics heretofore unattained by the use of ordinary papermaking furnishes.

In making the highest grade writing and printing papers, it has been the practice to use, as raw material, stable, white fibers, such as rag pulps or wood pulps of high alpha cellulose content derived from woods such as spruce. Because the fibers of such pulps are comparatively long, they interfelt well on the papermaking machine and, because they are free from non-alpha cellulose impurities, the resulting papers are resistant to the deteriorating action of air, heat and light, possessing what is known in the art as high permanency or good ageing qualities.

Before forming into paper, long-fibered stocks such as described must be treated in a manner to generate sufficient cellulose gel therein to impart the desired strength and folding endurance to the paper, as well as to reduce length of fiber sufficiently to result in a well-formed or "closed in" sheet. To attain these results, the papermaker subjects the stock to the action of a beater engine until it has acquired the desired gelatinized condition or slowness, and then passes it through a Jordan engine. The Jordan engine cuts the fibers and so conditions them for improved paper formation, but the shortened fibers do not offer as great resistance to tearing in the paper made therefrom as would the long-fibered stock if employed as a raw material.

In accordance with the present invention, a subordinate proportion of stable, white pulp of short fiber length is used along with long-fibered stocks such as hereinbefore described, as the use of such a mixture of fibers makes possible dispensing with or minimizing the use of a Jordan engine, and the production of well-formed papers of the desired strength, folding endurance, and of much higher tear resistance than that possessed by paper made from stock which has been passed through a Jordan engine. The short-fibered pulp which I employ may be derived from

short-fibered woods, such as poplar. It is essential that it be of high alpha cellulose content, as the use of a short-fibered raw material such as soda pulp is disadvantageous in the manufacture of high grade papers, 55 owing to its high proportion of non-alpha cellulose constituents, such as pentosans. The alpha cellulose content of the usual commercial soda pulp is only about 83% to 85%, and its pentosan content is about 8% to 15%, 60 which latter constituent, together with other impurities, renders the pulp unstable and unfit for use in high grade papers. The short-fibered wood pulp employed in the papermaking composition of the present invention 65 is of high alpha cellulose and low pentosan content. It may be prepared from short-fibered woods, such as poplar, by a process such as follows. The wood in chipped condition may be cooked in an acid sulphite liquor, 70

for instance in the usual calcium base liquor containing 1% combined and 5% free SO<sub>2</sub>, or in a sodium base liquor, to produce a cleaner and more easily bleachable pulp. The cooking operation may be carried out at 75 a temperature of about 275° to 285° F. for about nine to ten hours, during which time free SO<sub>2</sub> may be released from the digester to maintain the pressure at about 75 pounds. The digester contents may then be blown into 80 a pit, and the raw woodpulp may be separated from the spent liquor by washing in the usual manner. The raw pulp may be converted to a white product of high alpha cellulose content by suitable refining steps. 85 To this end, it may initially be treated at room temperature for about two to three hours, with a liquor containing about 1% to 3% chlorine or 1% to 5% hypochlorite bleach, based on the dry weight of pulp. Or, if 90 desired, both a suitable chlorine water treatment and hypochlorite bleach liquor treatment may be employed. The chlorine water and/or bleach liquor removes lignin and other coloring matter from the pulp, or renders such matter soluble in alkaline liquors. The pulp is then washed, whereupon it may be treated with an alkaline liquor to remove chlorine reaction products and other non-alpha cellulose constituents from the pulp. 95 100

For instance, the pulp may be treated at about 100° C. or at higher temperature and under super-atmospheric pressure for about four to six hours, with a solution containing about 5 10% to 12% caustic soda, based on the weight of dry pulp. Or, if desired, the treatment may be effected at lower temperature with a more concentrated caustic soda solution, for instance at from 20° to 40° C., for about two 10 hours, in a solution containing 50% caustic 15 soda, based on the weight of dry pulp. The refined pulp may then be bleached with a suitable agent to the desired whiteness, for instance, with calcium or sodium hypochlorite bleach liquor, preferably containing 20 sufficient free alkali to ensure a condition of distinct alkalinity throughout the bleaching 25 operation, as such a condition prevents the formation of oxycellulose and accordingly 30 results in a white product of maximum alpha 35 cellulose content and stability. If desired, a permanganate bleach liquor may be employed, in which case the liquor should be maintained neutral or acid, in order to avoid 40 degradation of fiber into oxycelluloses.

The resulting product is extremely free and resistant to gelatinization by beating, so that when mixed with long-fibered stocks such as rag pulp or long-fibered wood pulps, 30 and beaten, it retains its opacity and bulkiness and imparts these characteristics and better printing properties to the resulting paper. In either beaten or unbeaten condition, it shrinks and swells much less than do the 35 long fibers, and accordingly may be used to advantage in admixture with the long fibers to produce papers which undergo much less change in dimensions when exposed to varying 40 humidity conditions or when immersed in aqueous baths and then dried, than papers heretofore produced. This property of the fiber renders it especially valuable for use in the manufacture of blueprint and photographic papers, which are subjected to such 45 conditions.

In producing papermaking compositions, the short-fibered pulps may be added in desired proportion, say 10% to 25%, to suitable long-fibered stock, such as rag pulp or wood 50 pulp of high alpha cellulose content derived from long-fibered woods such as spruce, either before or after the long-fibered stock has been subjected to beating to produce cellulose gel in sufficient amount to impart 55 the desired strength and folding endurance to the resulting paper. Excellent results may be obtained when the unbeaten, short-fibered pulp is added after the long-fibered stock has been beaten to the desired slowness, 60 as in such case the short-fibered portion may be incorporated throughout the beaten and gelatinized long-fibered portion, with the beater roll sufficiently raised from the bed-plate of the beater engine to effect merely a 65 mixing of the fibers. The composition may

be run off into paper without being passed through a Jordan engine, to produce papers of excellent formation and having excellent stability, strength, folding endurance, tear resistance, bulk, and opaqueness.

I claim:

1. A papermaking composition comprising a stable, white, long-fibered pulp of high alpha cellulose content in gelatinized condition, and a stable, white, short-fibered wood pulp of high alpha cellulose content in free condition.

2. A papermaking composition, comprising a stable, white, long-fibered pulp of high alpha cellulose content and a subordinate proportion of stable, white, poplar pulp of high alpha cellulose content.

3. A process which comprises forming a mixture of stable, white, long-fibered pulp of high alpha cellulose content in gelatinized condition and stable, white, short-fibered wood pulp of high alpha cellulose content in free condition; and running off the mixture into paper.

4. A process which comprises beating a stable, white long-fibered pulp to the desired slowness; mixing a subordinate proportion of unbeaten, stable, white, poplar pulp therewith; and running off the mixture into paper.

5. A papermaking composition comprising a blend of two cellulose pulps, both being stable, white pulps of high alpha cellulose content, but one being derived from a long-fibered cellulosic source, and the other being derived from a short-fibered cellulosic source.

6. A papermaking composition comprising a blend of two wood pulps, both being stable, white pulps of high alpha cellulose content, but one being derived from a long-fibered wood of the type of spruce, and the other being derived from a short-fibered wood of the type of poplar.

In testimony whereof I have affixed my signature.

GEORGE A. RICHTER.

110

115

120

125

130